

May 1, 1934.

W. LINKE

1,957,279

HEAT ABSORBING WINDOW

Filed Nov. 10, 1930

FIG. 1.



FIG. 2.



FIG. 3.



FIG. 4.



FIG. 6.



FIG. 5.



Inventor. Walter Linke.

## UNITED STATES PATENT OFFICE

1,957,279

## HEAT-ABSORBING WINDOW

Walter Linke, Berkeley, Calif., dedicated to the  
People and the Government of the United  
States of America

Application November 10, 1930, Serial No. 494,707  
In Great Britain November 21, 1929

5 Claims. (Cl. 106—36.2)

This invention relates to means for eliminating the substantially dark heat from the whole radiation of a light source, but it differs from similar inventions already by its specialized object which consists in providing improved and less expensive window-panes destined for absorbing the dark heat specifically of the sun, (which is a body of a temperature unequalled by that of any terrestrial light source), and for transmitting as far as possible the light in amounts gradually increasing towards those rays of the spectrum for which the eye attains its maximum sensitiveness specifically at daylight intensities of illumination. While prior inventions relating particularly to window-panes only, for instance that of the British Patent 197,500, are quite suitable to fulfill the analogous purpose for the rays of artificial light, the panes of the present invention represent in fact an entirely 20 different article of manufacture, which would be inappropriate as a heat-filter in film projectors.

The invention comprises in the making of transparent or highly translucent heat-absorbing window-panes mainly the selection and controlled employment of those compounds of the chemical elements with atomic weights from 51 to 65 which are showing absorption bands in the vicinity of the one or the other end, and especially beyond the red end, of the visible spectrum, 30 and which have a relatively high transmissivity for the already mentioned luminous rays of the spectrum.

Reference is made to the drawing, wherein Figs. 1 to 4 represent various forms in which the invention may be employed, while Figs. 5 and 6 are explanatory diagrams.

Fig. 1 which needs no further description, shows the cross-section of a window-sash containing a solid pane in which the heat-absorbing compound is equally distributed, quite analogously to a pane made from any colored glass.

Fig. 2 representing the preferred form of the invention, shows a window-sash containing a pane of ordinary colorless glass, to the surface 45 of which the heat-absorbing substance is applied in the form of a preferably thin layer, indicated in the drawing by a black lining.

Fig. 3 shows a sash containing a heat-absorbing pane of the kind of Fig. 1, indicated by the 50 same manner of hatching, and

Fig. 4 a sash containing a pane of the kind of Figure 2, behind which in each of these cases a second pane of ordinary glass is arranged. The light is intended to come in all of these figures 55 from the left side.

Fig. 5 shows diagrammatically the difference between the spectral color luminosity of objects in bright daylight (a) and in poor daylight or under the average artificial illumination of interiors (b), and

Fig. 6 the spectral difference between the radiation of the sun (c) and of an artificial light source (d). Reference to these two figures will be made farther below in this description.

If the heat-absorbing compound is applied as 65 a thin layer to the outside surface of the pane, as exemplified by Figure 2, most of the absorbed energy is communicated by conduction and convection to the outside air, or is immediately re-radiated through the blue sky into the cold celestialspace.

Examples of performing the invention with the aid of a thin layer consisting of, or containing a material which fulfills the other requirements of the invention, are: glass flashed at its original 75 manufacture with a thin layer of such material in a vitrified condition; or glass coated on the outside with any varnish or lacquer or lac containing such material or substance in true solution or as a stain, or containing it in the form 80 of powdered glass or other vitreous or crystallic material, preferably of approximately the same refractive index as the coating; or a thin sheet or film of the specified properties glued to the glass-pane or fastened merely in contact therewith in the same frame. The absorbing layer may be applied by means of the transfer paper process, and, if composed according to ceramic principles, may be fused as a transparent glaze to the pane by firing afterwards. Two or more 90 layers with properties supplementing each other may be applied and fired simultaneously, especially if containing fluxes with melting points gradually ascending in such manner that the layer next to the pane melts first.

Artistic designs, applied by the said transfer paper process, or by hand by the glass painter, containing mainly coloring matters selected according to the principles of this invention, are within its scope.

Suitable compounds of the afore-mentioned group of chemical elements are found mainly among those of iron, copper, and nickel. The maximum of the most characteristic absorption band produced by iron is situated always around 105 0.001 or 0.0011 millimeter wavelength, and that of copper at 0.00085 millimeter (or  $0.25 \mu$ ) in the near infra-red. Nickel has in a large number of its compounds a band at 0.0007 in the red, and another band found in nickel glass at 0.0022 110

seems also to be caused by this element. Cobalt compounds in true solution will probably show in the infra-red the broad but shallow absorption band known from cobalt glass. Nickel and cobalt oxide in glass, of course, are of no use for the present invention, because their transmission is exceedingly low in the central part of the visible spectrum, except perhaps in the case of nickel oxide in strontian glass.

10 A plurality of absorbers with absorption-bands at different places in the infra-red, for instance the combination of an iron and a copper compound, will generally be a better absorber than a single compound in correspondingly higher 15 concentration alone. However, an absorber with a relatively low transmissivity in the center of the visible spectrum, or more accurately around 0.0005555 mm. wavelength, can be useful in this manner only in very minute and carefully controlled quantities.

10 A very important, though secondary condition of the present invention is that the light be as much as possible balanced, as it were, in order to give good and non-fatiguing vision. This is 25 accomplished by not only making the window-pane yellow-green but by also controlling its light absorption in such manner that the curve of the energy contents of the transmitted light slopes down gently and symmetrically to about 30 zero or any desired value at both ends of the visible spectrum. The balancing color by which it is intended to suppress partially the usually too abundant blue and violet rays must fulfill, of course, just as well as the original color, the 35 still more important condition of a high transmission around 0.0005555 mm. wavelength.

40 The selection of the balancing color depends, of course, entirely on the transmission curve of the heat-absorbers used. Uranium oxide and the various means for producing a yellow or light amber color in glass may be mentioned here as probably useful. A great many spirit and oil soluble dyes of yellowish or light brownish color will be useful in various varnishes and lacquers. 45 Only very small quantities of these balancing colors are necessary in most cases, and a combination of two or three dyes in varying quantities will be a very pliable means to enforce any desired absorption. The spectroscope is the best 50 means of disclosing the composition of the color, but in the case of the peculiar hue preferred for this invention a perfectly balanced transmission extending over the entire visible spectrum will also be indicated by the absence of dichromatism, 55 i. e. absence of a shifting of the dominant hue with the concentration of the absorber or the thickness of the layer. Practical experiments in most cases will lead more easily to the desired result than predetermining the absorption with 60 the aid of known transmission values.

65 Chromium and vanadium oxide in glass are known to suppress to a certain extent both ends of the spectrum simultaneously, though the blue end considerably stronger. Many organic dyes of green color will fulfill the same purpose in varnish and lacquer coatings, though generally freely transmitting the infra-red and also already the extreme red end of the visible spectrum. 70 A combination of two different dyes absorbing both ends of the spectrum separately will have the same or even a better effect, of course. If the substances used for suppressing the blue end contain iron, they can be presumed (with the caution which is always necessary where conclusions

75 from the color are drawn, or where the existence of a certain absorption band is generalized) to be heat-absorbing in spite of a yellow transmission color and in spite of having eventually their highest transmission in the extreme red.

80 If the absorption of the balancing color extends sufficiently far into the ultra-violet, and if it is embodied in a separate varnish coat outside over the other parts of the filter, this coat will protect the rest of the filter against the 85 weather and against the actinic rays of the sun. Such protection is advisable in any case for coatings made from celluloid solutions.

90 More definite advices for performing the invention are given in the following.

95 A manufacturer of colored glass has in all probability no other choice but to produce an iron and copper bearing glass by prolonged heating under oxidizing conditions. Many other means besides lead and boron are at disposal to shift the dominant hue of the glass more into the yellow-green (for instance sodium in iron silicates and in copper lead-silicates, further zinc and aluminum in certain cases), but no other efficient 100 heat-absorbers besides the oxides of iron and copper (and possibly vanadium oxide) in true solution in glass seem to exist for use with the present invention.

105 A glass painter, whose products are intended to be fired under oxidizing conditions, may be advised to use a suitably selected modification of the usual transparent glazes containing copper oxide. Boric acid should be employed in quantity just sufficient to secure a good transparency. The shifting of the hue into the yellow green may 110 be done by uranium oxide or better as much as possible by a yellow iron borate.

115 Very finely powdered glass in which iron oxide and copper oxide is contained in true solution, is the only heat-absorber I wish to recommend 11 at present definitely for use in various kinds of varnish coats. If for some reason the powder, or a combination of two powders, for instance a copper silicate and a yellow iron silicate of high 12 soda contents, is not applied simply in mixture with the varnish, one could proceed by dusting 13 it on a wet coat of varnish, the procedure to be repeated eventually once or twice after drying. As in most instances the indices of refraction of 14 glass and varnish are not very different, a semi-transparent coat with low diffuse reflection will 15 be obtained. By mixing a varnish of lower refractive index than glass with one of higher refractive index it is possible to produce a varnish 16 the index of which is equal after drying to that 17 of the powdered heat-absorbing glass. Eventually 18 the refractive index of the glass may be predetermined in a similar manner by varying 19 the composition of the glass. The knowledge of 20 the following figures, representing the indices of 21 refraction, will be useful for this purpose: Copal 22 resin and Canada balsam about 1.53, mastic 1.54, 23 amber and colophony (rosin) about 1.545, Peru 24 balsam 1.6, aloe resin 1.62, piperine (an alkaloid 25 which can be fused together with colophony and 26 other resins) 1.68, borax and boric acid (fused) 27 about 1.463, fused silica 1.4585, ordinary glass 28 (mean value) 1.52, light flint glass (36 percent 29 lead oxide) 1.575, glass painter's flux (78 lead 30 oxide, 22 silica) 1.89. The admixture of large 31 quantities of iron or copper oxides will probably 32 increase the refractive index of ordinary glass 33 quite considerably. Amber, hard copal, 34 and in the hands of an experienced man water

glass should be the most recommendable vehicles for the glass powder.

It is theoretically better to have the heat-absorbing substance in the layer in true solution or in a suspension of particles which is equivalent to a true solution, rather than relatively large particles, for instance of heat-absorbing glass, distributed in a vehicle, because then the indices of refraction of the absorber and of the vehicle

19 need not be equal. In order to attain this, it is necessary, in the first instance, that the absorber be soluble in one of the constituents of the varnish or lacquer. If this is not the case, an attempt must be made to find a substance which is

15 a common solvent for the absorber and the substance forming the finished sheet. In many cases the additional substance will be a volatile liquid which mixes with the solvent of the varnish or lacquer in the manner of a true solution,

20 as for instance water and alcohol, but which does not behave as water and oil with respect to one another. Ethyl acetate, for instance, is known to play this part in a great many cases. Further, during the evaporation of the solvent the absorber must not crystallize with such size of

25 grain that the transparency (or high translucency) is impaired. This necessity makes it probable that mainly dyes of high staining power are suitable for producing transparent lacquers,

30 and that the more complicated organic compounds of the mentioned metals, on account of their smaller inclination to crystallize, as dyes to be used in an evaporating solvent are for the present invention more suitable than the chemically simpler ones. Cuprammonium may be

35 mentioned as a heat-absorber which also is a solvent, (for cellulose). As example of heat-absorbers which the dyer is able to produce in a finished lacquer coat as a stain, may be mentioned the various copper compounds of acetic acid, nickel oxalate, and ferric ferro-cyanide.

Since there exist more than a hundred varieties of resins, lacs, and similar substances to be used in commercial varnishes, and since it is

45 known that the successful handling of every one of them requires some experience, I do not wish to make any definite suggestions for coloring these substances directly, (or without primarily coloring their solvents), except by the described

50 admixture of heat-absorbing glass powder of approximately the same refractive index. However, there can be no doubt that without further invention many so-called resinates and oleates with heat-absorbing properties are obtainable, or

55 are known to be obtainable, by fusing (or boiling) metal compounds with the varnish substances, or by precipitating the resinates in the known wet process. In the products variable

60 quantities of metal oxides are dissolved or compounded in a transparent state in the meaning of this invention, and their analogy with the so-called silicates, borates, etc., is obvious. While copper oleates seem to have generally an intensive green color, the resinates and oleates of iron

65 are generally of a yellowish or brownish color, so that they can be used for suppressing the violet end of the spectrum, besides in all probability contributing to the heat-absorption.

I do not claim any articles of manufacture showing an absorption in character quite different from the typical bands which appear when light is transmitted through the interior of compounds of iron, or copper, or nickel, and particularly if containing oxygen. This concerns especially copper and iron glasses produced under

reducing conditions, for instance Crooke's sage green (bluish green) glass or the heat-absorbing window-glass of the British Patent Specification 197,500. To avoid errors on the nature of the glass of this invention, it seems to be necessary to include here a short survey of the color of iron bearing glasses.

Small quantities of iron in a glass poor in oxygen and especially after quick chilling do not show a color corresponding to Beer's proportionality law of absorption, but are practically colorless, just as gold or copper glasses under the same conditions.

All glasses poor in oxygen must contain the iron necessarily in the elemental metallic state, because the process of their production is identical with the process of reducing iron ore. Small iron contents of one or only a few percent of the metallic element seem to give the best blue color. The selective absorption caused by colloidally suspended metal particles in glass is in character very much different from that caused by substances in true solution, and consists mainly of extended regions of more or less uniformly low transmission, which in certain cases is nearly the exact reversal, or the complementary color, of the absorption of thin metallic films of the same substance. Tin, zinc, and cadmium, which all are metals of high soldering and alloying power, have become known as promoting the blue colloidal gathering of the iron molecules.

Glasses poor in oxygen and rich in iron particles, which in this case are probably much larger than in the former cases, are smoky grey or black, and especially in the latter case appreciably magnetic.

Only glasses rich in oxygen are able to contain the iron as a proper glass constituent. Their color is usually green or yellow-green, but may become displaced, by the influence of boric acid or other glass constituents, towards the yellow or even into the red. It is this green or yellow green form of oxidized iron glass which is quite exclusively used as an absorber for the present invention, as far as iron in glass is concerned, and which alone shows a high transmissivity for yellow green light in combination with an infrared absorption band of sufficient depth and broadness. High and prolonged heating under oxidizing conditions is necessary to form a proper iron silicate. By the oxidation the glass of this invention becomes in substance as different from the prior heat-absorbing glasses of blue and blue-green color as oxidized green copper glass is different from reduced red copper glass made from the identical batch, though in the case of iron glasses the difference in color is not so striking.

Ferric oxide ( $Fe_2O_3$ , polishing rouge, crocus) shows already in the dry state differences of color which are caused merely by the size of the grains of the particular variety. The same is the case when the oxide is distributed in the glass undissolved or only partially dissolved, and able glass painters understand how to produce a large variety of rather different colors merely by the proper selection of the oxide and the flux and by controlling the time and temperature of heating. The hard ferric oxide seems to dissolve less easily than other iron compounds, and a fused soda or other flux seems to be much less suitable for its dissolution than a glass in statu nascendi. Such non-metallic elements as arsenic, chlorine, selenium, which are of electro-negative character, or of negative valency, have a strong tendency to collect the iron and other coloring elements

80

85

90

95

100

105

110

115

120

125

130

135

140

145

150

from the less stable compounds and especially from the already existing colloidal particles and, upon vaporizing, to take them entirely out of the glass into the chimney. While the freedom of the original batch from "decolorizing" materials or impurities of such electro-negative character appears to be necessary in order to keep the coloring materials in the mixture until after melting the respective colored silicates are formed, the use of arsenic in large pieces thrown into the molten glass, where it sinks to the bottom and quickly vaporizes, will remove generally only the remaining undesired colloidal impurities. However, by too much of it also a considerable part of the colored silicates used in this invention, among which the true iron silicate is probably the most stable, may be destroyed again.

The color of glass containing the ferric oxide in larger particles of still entirely ultra-microscopic size can be presumed to be in character similar to that of polishing rouge. This means that the high transmissivity at the extreme red end of the visible spectrum continues into the infra-red to at least 0.0044 mm. wavelength, so that a glass containing the iron solely in the colloidal ferric state would be heat-transmitting for every practical purpose.

Iron glasses of amber color, in which reduced iron is accompanied by reduced carbon or sulphur, or oxidized iron by oxidized manganese, are not considered to be heat-absorbers in the meaning of this invention, because it is the very nature of any amber color that it has its highest transmissivity in the red and shows a continuous or even gradual decrease towards the violet. This is irreconcilable with the principle of this invention, of providing in the yellow-green a transmissivity as high as possible, accompanied by a low transmission in the red and beyond. Only, if the amber color is very light, it may be used occasionally for subduing the violet rays too abundantly transmitted by most copper glasses, though not only an easily procurable yellow or greenish yellow iron glass with a pronounced heat-absorption but even any light yellow glass (which in contrast to the amber glass has an equally high transmission for all long waves, including the yellow-green) would be in any case more adequate for this purpose.

A smaller or larger part of the iron is probably in every glass unintentionally or unavoidably present in the form of dissolved ferric oxide, or of a so-called iron silicate. As compared with this uncontrolled occurrence of dissolved ferric oxide the present invention comprises the use of glass in which the ferric oxide is contained predominantly in true solution, and intentionally, as a regular manufacture.

Sheets consisting of relatively opaque and light-diffusing material are not within the scope of this invention, regardless of whether heat-absorbing or not. A reflecting layer may be combined, however, in a novel manner with the invention by applying on the outside over the transparent heat-absorbing layer a semi-opaque white coat which partially reflects and partially transmits the light in a diffused manner. The reflected part of the light does not intrude in this case the clear absorbing layer at all, while, when the white reflecting layer is applied behind the absorbing layer, an additional amount of radiation is absorbed by the repeated passing of the undesired and reflected light through the absorbing layer, so that the pane becomes considerably hotter than

in the first case, or even than without any reflecting layer.

The intermediate case, in which a white (including infra-red reflecting) pigment is embedded in the clear heat-absorbing layer of my invention, is also within the scope of my generic claims.

Water soluble coatings, and water soluble absorbers therein, while not objectionable as filters for artificial light sources in certain cases where no exposure to the weather or to the touch of human hands is intended, are deemed to be unsuitable for the present invention.

The improvements constituting my invention are not intended to go beyond the limits of physical and physiological optics including those of invisible radiation in the neighbouring parts of the visible spectrum, and, as I have not had, till now, any occasion to work the invention out practically, my advice as that of a layman in chemistry and in the art of the dyer, cannot be infallible, and, therefore, is intended only to indicate the direction in which other heat-absorbing materials, besides heat-absorbing silicates and the like, and processes for producing the same are at the disposal of any expert in chemistry.

The following physical and physiological data, and the conclusions drawn therefrom, not only form to a large part the foundation of my invention, but also indicate the preferred manner of its performance.

One and the same amount of radiant energy in the form of good or average daylight illumination by windows, producing within the room by absorption in every case the same amount of heat, will incite in the average eye the maximum amount of luminous sensation when consisting of light of 0.0005555 mm. wavelength (yellow-green). Light of 0.000533 and 0.000570 mm. (near both ends of the yellow-green region) will incite only 90 percent thereof, light of 0.000510 (at the border between yellowish and bluish green) and 0.000614 (orange-yellow) only 50 percent, and light of 0.000475 and 0.000652 mm. only 10 percent of the mentioned maximum sensation. These wavelengths are so chosen that the curve of luminous efficiency of good daylight may be easily completed on paper by making it practically zero at 0.0004 and 0.00072 mm., though it extends for most persons in minute traces at least until 0.000397 and 0.000760 mm., where the H and A lines of the solar spectrum were discovered visually. These figures are valid only for at least the illumination intensity of daylight interiors, which can be taken roughly as 10 millilambert (one millilambert being the thousandth part of a lambert, or of the brightness of a perfectly white and perfectly diffusing surface illuminated by the standard sunshine of 10000 meter-candles), while the average illumination of night interiors is roughly 0.1 millilambert. Below 10 millilambert, especially within the relatively narrow range between 1 and 0.1 millilambert, however, the maximum sensitiveness of the eye shifts rapidly from 0.000555 to 0.000510 mm. wavelength, but seems to move thereafter even for very much lower intensities only slightly farther. The last named figure, on account of its smaller importance and of the more complicated conditions of research has been ascertained only with incomparably less accuracy than the figure for good daylight illumination.

There seem to exist inner reasons why this range is identical with that unique region of the spectrum for which no single complementary color exists, because it is not green enough to 150

be complemented by red, and not yellow enough to be complemented by violet.

Further, the non-monochromatic color corresponding to any wave-length of the said region 5 seems for that illumination intensity, for which this hue functions as maximum of luminous efficiency, to be the only one which allows such spectral distribution of its energy that the corresponding luminosity curve declines symmetrically 10 unto the extreme limits of visibility in the red and violet, and which then will not show dichromatism, or a shifting of its hue, with increasing or decreasing saturation of the coloring agent. Any other color could be made free from dichromatism only by suppressing a more or less considerable region at one of the ends of the spectrum 15 entirely.

Fig. 5 shows the luminosity curves of the best possible (a) and of that poorest daylight illumination (b) at which a change to artificial illumination should be made. While the wavelength of 20 0.0005555 mm., or  $0.556\mu$ , which is marked in this figure as the maximum of one of these two curves, is the primarily preferred hue for this invention, 25 with any greenish yellow hue included as a less efficient equivalent, the wavelength of 0.000510, or  $0.510\mu$ , which is marked in the figure as the maximum of the other curve, and which separates the yellowish green from the bluish green, 30 is deemed to be the natural border line of the invention towards the short-waves.

As a standard for the color work involved in the present invention I recommend three solutions of 57.52 grams of cupric chloride, 1.22 grams 35 of potassium bichromate, and 8.22 grams of ferric chloride, respectively, dissolved in each case in 1000 cubic centimeters of distilled water, and filled in three successive cells of colorless material, each 40 of 1 centimeter inner width. If instead of these cells rectangular bottles of, for instance, 1.5 centimeters width would be used, the solutions would have to be diluted proportionally, using in this case 1500 ccm. of water instead of 1000. This threefold filter, as originated by Karrer for photometric work, has a curve of spectral transmission 45 which very closely approaches the luminosity curve of radiation as found already with ample exactitude by the earlier work of Ives, with a maximum around a wavelength of 0.00055 mm. or 50 slightly more.

Fig. 6 illustrates the difference between the radiations of the sun (c) and an artificial light source (d), or more exactly the radiations of two perfect black bodies of 6000 and 2000 centigrades above the absolute zero of temperature. The areas under the two curves are intended to be 55 roughly equal, thus representing equal energy or equal heat. It is already from this figure apparent that for the two light sources different requirements will have to be fulfilled by filters for 60 the same, and the nature of these requirements is set forth more clearly in the following.

The distribution of energy in the solar spectrum was found in the city of Washington on 65 the average as follows, when the sun was 30 degrees above the horizon (arbitrary units): 130 at 0.0004 mm. in the violet, 323 at 0.0005, 306 at 0.0006, 268 at 0.0007 in the red, 141 at 0.001, 55 at 0.0015, and 21 at 0.002 mm. For the sun 70 standing in the zenith and for high altitudes above sea level the violet and ultra-violet component of the energy curve increases very considerably, but the near-infrared component only very slightly. Further, in the regions near the 75 equator the air contains according to Hann on

the average 2.63 percent water vapor, at 50 degrees northern latitude 0.92 percent, and at 70 degrees only 0.22 percent. It is well known that water vapor begins to absorb at 0.0015 mm. in the infra-red, and that the presence of large quantities of it allows scarcely any transmission beyond 0.0022 mm. These conditions must cause that the infra-red energy of the sun is in the tropics still more concentrated near the visible end of the spectrum than the figures given above indicate. 80 88

While the sun is a body of a temperature of probably more than 5500 degrees Celsius, the maximum of the radiation of which, after transmission through the atmosphere, coincides on the average probably with the wavelength of maximum luminous efficiency, the light sources of film projectors, according to a temperature scarcely half as high, and according to the specific emissivity of tungsten radiate their maximum energy in the infra-red and at a wavelength about three times as long. The ceasing of the sun's infra-red practically at 0.0022 mm., or in the tropics, where much water vapor though little real moisture is contained in the air, eventually already at 0.0015, 90 makes it possible to select appropriate heat-absorbers for this invention not only from a much larger number of substances, but also according to a different principle, according to which copper compounds on account of the proximity of 95 their absorption band to the visible spectrum must be rated rather high. By the earlier researches of Crookes, who by the use of black biotite mica isolated mainly the heat waves of a length of more than 0.0015 mm., only the 100 particular suitability of filters for artificial radiation sources was tested, and as is well known, no other efficient absorber besides glass containing iron in the reduced state was found. 105 110

The properties required from the window panes 115 of the present invention are in the visible part of the spectrum perhaps still more different from those required from filters for artificial light sources, and particularly of cinematographic projectors, than in the infra-red.

According to the measurements of Allen (Phys. Rev., vol 11, 1900, p. 257) it is necessary for flashes of long waved light at low illuminations to follow each other much more rapidly than flashes of blue light if the eye is not to perceive flicker. At 120 that intensity of illumination at which the phenomenon had its maximum it was necessary for flashes of yellow-green light to follow each other two and a half times as rapidly as flashes of blue light. Since not only a shifting of the hue particularly into the yellow-green, but also any increase of the intensity of illumination causes more flicker, it is clear that one condition for the desirable increase of brightness of the picture on the screen as rendered by the standard film 125 of 16 pictures per second and by the present type of apparatus, is the avoiding of a high transmission specifically in the yellow-green. 130 135

Not only is the average brightness of the various parts of a moving picture on the screen 140 probably even below the average brightness of night interiors of roughly 0.1 millilambert, but the picture occupies in general also only the smaller part of the retina, so that the eye becomes adapted to a mean between the brightness 145 of the picture and the general brightness of the other parts of the room, which is illuminated mainly by the reflex from the screen. It has been shown already that for an active brightness of less than 0.1 millilambert the maximum sensi- 150

bility of the eye shifts beyond 0.000510 mm. wave length, and this is one more reason why any efficient light filter for film projectors must be of a far more bluish color than if it had only the purpose of suppressing the too abundant red and yellow rays of a tungsten filament.

I wish to include in the scope of my invention also the intermediate articles of manufacture specifically prepared and compounded for the same, as for instance filters and colored materials the absorbers of which are selected for their high transmissivity in the yellow-green, though their transmissivity in the neighbouring parts of the spectrum may be still slightly higher, and which filters and materials it is intended to use together with another filter for suppressing those too abundant rays. In former inventions concerning heat-absorbing windows the color was not considered at all, so that an absorption band situated right in the yellow-green would not have been a principal objection (or was even desired, as in the German Patent 160,356, where it is proposed to transmit only the blue and the orange-yellow rays in order to obtain a neutral white of relative coolness). In the present invention, however, at least as much regard to a (non-monochromatic) transmissivity centered in the yellow-green is taken as to the regard to a high luminosity of the transmitted energy, so that the fulfillment of the latter regard is in general hampered by the former regard to a certain quality of the luminosity. The following example will make this clear. If a composition of the transmitted energy corresponding to that of the threefold filter recommended above as a standard were desired or demanded, and a certain hypothetical filter or absorber would transmit besides 100 percent of the yellow-green light also 100 percent of light of 0.000475 mm. wavelength, then according to the prescribed energy curve only 10 percent of the transmitted energy of the latter wave-length with a luminosity value of only 1 percent can be counted as fulfilling the requirements of the invention in this case, and the superfluous 90 percent of blue light have to be suppressed by another absorber or filter.

It must be presumed that the iron glass and the copper iron glass of this invention has been used already before as a colored glass for the purpose of art and decoration in windows, or that the same or similar glasses have been tried also as light filters in film projectors. However, it has been shown hereinbefore already that the absorption requirements (in the infra-red) as well as the transmission requirements (in the visible spectrum) of the present invention are different from those of other inventions.

There is further not only the difference in size between a window-pane and a filter for a small film picture of at most one inch side length, which difference has already a slight influence on the methods of manufacture, but the high concentration of the heat in the latter case on a small area makes the obtaining of a low coefficient of heat expansion by the use of high boron and low soda contents imperative. The high acidity, or borate forming power, of boric acid, and the fact that iron borates as well as highly alkaline soda lime silicates are of yellow color, then shows again the necessity of employing different methods for obtaining the adequate transmission and heat-absorption for each of the two different purposes.

Comparative tests as to the specific efficiency

nous transmission as judged by the eye can be made by observing the quickness of the rise within the first minute or other short time unit, or the total rise after a sufficient time, of a thermometer with blackened bulb placed behind the samples. In connection with the present invention only the sun can be used as an energy source for experiments.

There exists a critical point beyond which in the case of this invention the selective absorption should never be augmented. When increasing the quantity of heat-absorbing substance per surface unit, the ratio between the luminous effect on the one hand, and the energy which becomes stationary within the room on the other hand, will reach a point beyond which human comfort and efficiency becomes smaller again, because the window glass by becoming hotter with growing absorption would hinder a decrease of the temperature sufficient to compensate for the increasing loss and the increasing color saturation of the light. The maximum color saturation of the panes of my invention is probably especially in those cases considerably lower than the average saturation of colored glass made for art and decoration, in which a heat-absorbing layer is provided on the outside of the pane, and in which the size of the windows has been restricted already originally by reason of the costs of glass, or in order to limit the entrance of heat.

The main argument usually brought forth against heat-absorbing windows is that after a while the pane itself becomes warm and then communicates its heat in secondary form by radiation and air convection to the room. It can be shown, however, that in any case by far the larger part of the heat is disposed off towards the outside, and that the room can be protected further from the heat of the pane by providing the heat-absorbing substance in the form of a thin layer on the outside of the pane, as in Figure 2, or by placing a second sheet of ordinary glass behind the absorbing pane, as in Figure 3, or by combining these means, as in Figure 4.

Not only in the case of Figures 3 and 4, in which a second sheet of ordinary glass is placed behind the absorbing pane, but also in the case of two panes of ordinary glass, as often used in cold climates, it is valuable to know that the airspace between the two panes should not be made too wide, as it is usually done. As the result of various researches (Smithsonian Physical Tables, tables 286 and 287) it was found that at ordinary temperature differences only in spaces up to fairly exactly one half of one inch practically no air circulation at all takes place, and that the heat is transferred in this case only by conduction in quantities proportional to the width of the space. In vertical spaces of greater width than one half of one inch the viscosity of the air is not sufficient to hinder the establishment of a current which conveys, however, the less heat from one side to the other the higher the space, because its swiftness does not increase as fast as the height of the space, probably on account of rapidly increasing energy losses by eddies where the current is forced to change its direction. The influence of these eddies decreases, on the other hand, with the width of the space, so that a critical width exists which can not be surpassed without losing more heat by the more rapid air circulation than is gained by the increased conduction resistance of a wider gap. The following minimum values of transferred heat (conduction and convection) in gram calories per

square centimeter per hour per each degree Celsius of the temperature difference of the two surfaces forming the space have been found, after allowing for radiation, for the following most effective widths:

- 0.250 calories at 1.4 cm. width in a space 10 cm. high,
- 0.167 calories at 1.6 cm. width in a space 20 cm. high,
- 10 0.112 calories at 2.5 cm. width in a space 60 cm. high.

There are reasons to assume that in a space of slightly more than one half inch width the up and down current has the form of a very thin sheet flowing over the surface of the warm and the cold pane, and that by the collision of scattered air between the two currents always a core of practically still air of the fairly constant thickness of one half inch remains, no matter how wide the space. Consequently I believe that the actual conditions can be well represented by the following rule according to which the most effective width of the space between two window panes is for all practical sizes equal to one half of one inch plus one fiftieth part of the height of the panes.

The superiority of yellow-green eye protective glasses for augmenting visual acuity and for diminishing eye fatigue in bright sunlight has been ascertained by M. Luckiesh (Color and its Application, p. 154 ff) beyond doubt. Yellow-green eye glasses are not necessarily infra-red absorbing. Occasionally one and the same author advocating eye glasses of this color can be found to deny the feasibility or usefulness of heat-absorbing windows. In fact, however, it is only a paradox that in an effective heat-absorbing window just the hottest part of the spectrum has to be transmitted.

There exists no natural standard of color at all. If only that trifling quantity of blue and red rays above a certain threshold value for inciting the sensation of color of the objects in a room is contained in the light, the complex of color with respect to the light itself is excluded in the mind, and in the case of green light only the conceit of that coolness arises of which it is not only suggestive, but which mostly is its real and physical property. The light in a room equipped with heat-absorbing windows of the proper color is in character identical with that under a green foliage or in a green bower, which from hereditary reasons can be considered as the most natural human sojourn since the almost recent time when the earth was covered nearly everywhere with primeval forest.

I claim:

1. Transparent and highly translucent sheets and layers, and materials representing intermediate articles of manufacture for making the same, for selectively transmitting specifically the radiation of a body of a temperature of more than 5000° centigrade, characterized by containing a coloring matter of non-colloidal nature, obtained under non-reducing conditions, which matter is selected for exhibiting in combination with the

other constituents of the transparent material strongly an absorption band having its influence mainly in the red and the near-infrared of wavelengths shorter than 0.0015 millimeter, and for having under the same conditions a relatively high transmissivity in that central part of the spectrum of wavelengths longer than 0.00051 millimeter, for which no single complementary hue exists in the spectrum, and which coincides with the range of the Purkinje effect for illuminations of daylight intensities.

2. Transparent and highly translucent sheets and layers, and materials representing intermediate articles of manufacture specifically prepared and compounded for making the same, for the purpose of selectively transmitting the radiation of a body of a temperature of more than 5000° centigrade, characterized by containing a transparent compound, obtained under non-reducing conditions, of a chemical element with an atomic weight between 55 and 64, which compound is selected for strongly exhibiting the absorption band of the respective element in the near infrared and for having a high transmissivity in the greenish yellow and yellowish green region of the spectrum, and by containing as a further addition a substance for subduing the transmission on the shortwaved side of this spectral region.

3. Transparent and translucent sheets and layers, and materials specifically prepared and compounded for making the same, containing several of the elements iron, nickel, cobalt, copper in the form of transparent compounds selected for exhibiting the typical absorption band of the respective elements in the near infra-red and for having a relatively high transmissivity in the greenish yellow and yellowish green region of the spectrum unto 0.00051 mm. wavelength, for the purpose of selectively transmitting specifically the radiation of a body of a temperature of more than 5000° centigrade, as set forth.

4. A colored glass for selectively transmitting the radiation of a body of a temperature of more than 5000° centigrade, characterized by containing the silicates of iron and copper, obtained under oxidizing conditions, all the constituents of the glass being selected as to their nature and quantity for producing by their coaction strongly the typical absorption bands of iron and copper silicates and for having a high transmissivity in the yellow-green region of the spectrum of wavelengths longer than 0.00051 millimeter.

5. A colored glass made specifically for the purpose of selectively transmitting the radiation of a body of a temperature of more than 5000° centigrade, as set forth, characterized by containing the oxide of at least one of the elements iron and copper together with the oxide of at least one of the elements chromium and vanadium, all the constituents of the glass being selected as to their nature and quantity so as to produce by their coaction strongly the characteristic absorption bands of the proper silicates of the respective elements, and to exhibit the highest transmission in the yellow-green of the spectrum at a wavelength longer than 0.00051 millimeter.

WALTER LINKE.